

## UNITED STATES PATENT OFFICE

FREDERICK C. NONAMAKER, OF GLOUCESTER CITY, NEW JERSEY, ASSIGNOR TO WELS-BACH COMPANY, OF GLOUCESTER CITY, NEW JERSEY, A CORPORATION OF NEW JERSEY

## LUBRICATING AND SEALING FLUID

No Drawing.

Application filed March 9, 1927. Serial No. 174,104.

The present invention relates broadly to the art of lubricating and sealing fluids adapted for use in compressors and similar apparatus, and more particularly to a fluid 5 of this character especially adapted for use in refrigeration systems.

In refrigeration systems of the type commonly in use at the present time, there is utilized a mechanical pressure-producing 10 means usually designated as a compressor and effective for producing the desired pressure conditions on the gaseous refrigerant. Considerable difficulty has heretofore been experienced in the operation of such compressors in preventing either the leakage of the refrigerant under pressure outwardly through the stuffing box or boxes or the leakage of air inwardly into the system. The first condition is objectionable due to the loss 15 of refrigerant, and the second condition is objectionable not only because it produces a continuously changing condition within the system, but because it increases the moisture present in proportion to the amount of moisture in the air drawn in. In an effort to overcome this condition, it has heretofore been proposed to provide a lubricating and sealing fluid effective for maintaining a constant seal on the compressor. While a large number of 20 different liquids and compositions have been proposed for this purpose, it has been found that particularly beneficial results are obtained by a mixture of glycerine and ethylene-glycol. Both of these ingredients are 25 members of the alcohol series, glycerine being a tri-hydric alcohol and glycol a di-hydric alcohol. The combination is of advantage since glycerine alone has high viscosity at low temperatures, thereby requiring a high 30 watt load on the motor which drives the compressor in starting. Glycol alone possesses practically no lubricating properties, and therefore, could not be used exclusive of some lubricant. These ingredients have been combined in the proportion of substantially 79% 35 glycerine to 21% of glycol.

In the use of compressors employing such a lubricating and sealing material, I have observed a deposit in the system, and particularly in the compressor parts, which deposit

very much resembles a copper deposit. It has heretofore been assumed by those skilled in the art that a chemical reaction takes place in systems of this character by reason of which copper was deposited from the coils 55 onto the various ferrous parts. I have found, however, that this compound is due largely to oxidation of ferrous material in the presence of the water in the system. A glycerine-glycol combination possesses extremely deliquescent properties and rapidly absorbs moisture, this moisture being effective for oxidizing the ferrous materials as set forth.

In some cases, the deposit has become so 60 pronounced as to produce objectionable binding of the compressor parts, seriously interfering with the efficiency of the system and resulting in actual deposition on such parts to an extent preventing effective operation. 65

Of the refrigerants utilized at the present time, sulphur dioxide and ethyl chloride are the most important in apparatus of the expansion type. With either of these refrigerants, or in refrigeration systems generally, 70 it is desirable to prevent the production of an acid condition, as such acid condition reacts destructively on the operating parts, and in many cases is as objectionable as the oxidation, of the character referred to, it- 75 self. As the result of a series of experiments, I have found that while the oxidation may be prevented by the application either of acid compounds or of compounds resulting in the production of an acid condition, such a treatment is objectionable for the reasons referred to. In accordance with the present invention, therefore, I propose to utilize in a lubricating compound a reagent preferably 80 of an alkaline nature having either actual reducing properties, where it is to be added to systems which have been in use for some time, or having properties inhibiting oxidation where intended for use in freshly installed systems. 85

I have found that reagents effective for this purpose and having alkaline characteristics as referred to may be chosen from a large number of different groups, including sulphides and sulphites, thiosulphates, com- 90 95 100

pounds of the phenol group, such as pyrogallol, which is a tri-hydric phenol, and compounds in which the hydroxyl radical is present. Where ethyl chloride is utilized as a refrigerant, sulphides are objectionable by reason of the odorous compounds which they produce with the ethyl chloride, mercaptans or substances similar thereto resulting therefrom.

In all cases, it is desirable that the reagent utilized be soluble in the lubricating and sealing fluid, and for this reason, potassium sulphite is much more effective than sodium sulphite, although either may be utilized in accordance with the present invention. When the thiosulphates are utilized, I have found that the sodium thiosulphate is sufficiently soluble to permit its use.

The present invention contemplates, therefore, the mixture with a lubricating body of the alcohol series, and preferably comprising a tri-hydric alcohol, such as glycerine, and a di-hydric alcohol, such as glycol, of an ingredient or reagent soluble therein and acting to prevent oxidation. I am not aware that heretofore in the art, it has been proposed to combine with a lubricating and sealing fluid an ingredient or reagent effective for either reducing or inhibiting oxidation. Certain advantages of the present invention, therefore, arise broadly from the addition to a lubricating and sealing fluid, capable of use in refrigerating systems, of an ingredient or reagent having the characteristics referred to.

It will be apparent that the amount of the ingredient added in accordance with the present invention may vary in accordance with whether use is made of it in a new structure in which oxidation has not occurred, or in an old structure in which considerable oxidation has already manifested itself. In the first instance only slightly more than a trace of the oxidation inhibiting ingredient is required, while in the latter case, the percentage may vary from a trace up to a substantial amount. Although acid reagents may be utilized as herein pointed out, the alkaline reagents are preferable under most conditions. One example of a mixture which may be utilized in accordance with the present invention comprises 70 to 80 per cent. of glycerin, 20 to 30 per cent. of glycol and from a trace to 5 per cent of sodium sulphite. If potassium sulphite is utilized, the percentage may be increased. Substantially the same percentages may be utilized when the inhibiting ingredient comprises either sodium or potassium thiosulphate.

Still other advantages of the invention arise from the addition to a lubricating and sealing fluid of an ingredient or reagent of alkaline characteristics and preferably soluble in the lubricating compound being utilized.

Still other advantages of the invention arise from the provision of a lubricating compound having dissolved therein an ingredient or reagent of such nature as not to produce with the refrigerant an objectionable odor.

I claim:

1. In a lubricating compound, a lubricating body comprising glycerol and glycol having sodium thiosulphate in solution therein effective for reducing oxidation. 75

2. In a lubricating compound, a lubricating body of the alcohol series liquid at normal temperatures having sodium thiosulphate in solution therein effective for reducing oxidation. 80

In testimony whereof I have hereunto set my hand.

FREDERICK C. NONAMAKER.

85

90

95

100

105

110

115

120

125

130